

# United States Patent [19]

Sugita et al.

[11] Patent Number: 4,819,395

[45] Date of Patent: Apr. 11, 1989

[54] TEXTILE REINFORCED STRUCTURAL COMPONENTS

[75] Inventors: Minoru Sugita; Teruyuki Nakatsuji; Tadashi Fujisaki, all of Tokyo; Hisao Hiraga, Yokohama; Takashi Nishimoto; Minoru Futagawa, both of Sagamihara, all of Japan

[73] Assignees: Shimizu Construction Co., Ltd., Tokyo; Dainihon Glass Industry Company Ltd., Sagamihara, both of Japan

[21] Appl. No.: 69,483

[22] Filed: Jul. 2, 1987

Related U.S. Application Data

[63] Continuation-in-part of Ser. No. 894,832, Aug. 8, 1986, Pat. No. 4,706,430.

[30] Foreign Application Priority Data

Dec. 26, 1985 [JP] Japan ..... 60-295751  
Feb. 26, 1986 [JP] Japan ..... 61-41197

[51] Int. Cl. 4 ..... E04F 15/10; B32B 3/10; F16B 2/14

[52] U.S. Cl. ..... 52/309.16; 52/660; 428/109; 156/181

[58] Field of Search ..... 156/181; 428/109, 113, 428/255; 52/309.16, 660-662

[56] References Cited

U.S. PATENT DOCUMENTS

|           |         |                    |           |
|-----------|---------|--------------------|-----------|
| 719,489   | 2/1903  | Miquel .....       | 52/660    |
| 1,080,221 | 12/1913 | Jester .....       | 52/661    |
| 1,123,304 | 1/1915  | Jester .....       | 52/660    |
| 3,734,812 | 5/1973  | Yazawa .....       | 428/109   |
| 3,755,054 | 8/1973  | Medney .....       | 156/181   |
| 4,144,371 | 3/1979  | Okie et al. ....   | 428/255   |
| 4,448,832 | 5/1984  | Kidwell .....      | 428/113   |
| 4,706,430 | 11/1987 | Sugita et al. .... | 52/309.16 |
| 4,715,560 | 12/1987 | Loyek .....        | 428/113   |

Primary Examiner—James L. Ridgill, Jr.

Attorney, Agent, or Firm—Oblon, Fisher, Spivak, McClelland & Maier

[57]

ABSTRACT

A textile reinforced structural component including: a structural component body made of a structural filler; first parallel textile elements; second parallel textile elements crossing the first parallel textile elements at first crossing portions, each of the first textile elements and the second textile elements including at least one row of first textiles and a first resin matrix, made of a first resin, for bonding the first textiles; and an attaching mechanism for attaching the first reinforcement elements and the second reinforcement elements at corresponding first crossing portions to form a grid member. The attaching means includes the first resin. The first and the second reinforcement elements are impregnated with the first resin before attachment thereof, and the grid member is embedded in the structural component body.

17 Claims, 12 Drawing Sheets





FIG. 1



FIG. 2

FIG. 3



FIG. 4



FIG. 5



FIG. 7



FIG. 8



FIG. 9

FIG. 11



FIG. 10



FIG. 12

FIG. 13



FIG. 14



FIG. 15



FIG. 16



FIG. 17



FIG. 18



FIG. 19



FIG. 20



FIG.21



FIG.22



FIG.23

FIG.24



FIG.27



FIG.28



FIG.25



FIG.26



FIG.30



FIG.29



## TEXTILE REINFORCED STRUCTURAL COMPONENTS

### CROSS REFERENCE TO RELATED APPLICATION

This is a continuation-in-part of our application Ser. No. 894,832 filed Aug. 8, 1986, now U.S. Pat. No. 4,706,430, issued Nov. 17, 1987.

### FIELD OF THE INVENTION

The present invention relates to textile reinforced structural components such as textile reinforced walls, girders and columns of a concrete construction, a body of a fiber-reinforced plastic boat and the like.

### BACKGROUND OF THE INVENTION

U.S. Pat. No. 4,578,301, the disclosure of which is hereby incorporated herein by reference, discloses a typical example of the prior art fabric reinforced cement structure, in which a reinforcement, consisting of a plurality of mesh textile fabric layers, is embedded in a matrix of water hardenable material such as a portland-cement-based mixture. Each layer includes two crossing sets of straight laying parallel textile elements which may be united by bonding to form the fabric. The individual textile elements may be monofilaments, spun yarns, bundles, etc. This prior art reinforcement is disadvantageous in that it is relatively small in bonding strength of the crossing sets of parallel textile elements, and in that rather large thickness is necessary to reinforce the matrix.

### OBJECT OF THE INVENTION

Accordingly, it is an object of the present invention to provide a textile reinforced structural component which provides sufficient strength to the matrix with a fairly small thickness as compared to the prior art reinforcement.

### SUMMARY OF THE INVENTION

With this and other objects in view, the present invention provides a textile reinforced structural component comprising: a structural component body made of a structural filler; first parallel reinforcement elements; second parallel reinforcement elements crossing the first parallel reinforcement elements at first crossing portions, each of both the first reinforcement elements and the second reinforcement elements including at least one row of first textiles and a first resin matrix, made of a first resin, for bonding the first textiles thereof; and attaching means for attaching the first reinforcement elements and the second reinforcement elements at corresponding first crossing portions to form a grid member, the attaching means comprising the first resin, wherein the first and the second reinforcement elements are impregnated with the first resin before attachment thereof, and wherein the grid member is embedded in the structural component body.

Preferably, at least one of both the first reinforcing elements and the second reinforcing elements may each comprise a plurality of textile rows. The textile rows of both a corresponding first reinforcing element and a corresponding second reinforcing element are alternatively stacked at the first crossing portion. The first reinforcing elements and the second reinforcing elements are bonded with the first resin at the first crossing portions. Such a structure provides the grid member

with excellent strength as well as a substantially equal covering depth of the matrix material over the first crossing portions.

In a preferred form, the grid member may include 5 first resin impregnated mesh textiles and second resin impregnated mesh textiles. Each of the first and second resin impregnated mesh textiles may pass through at least one of both first reinforcement elements and second reinforcement elements to form a mesh in each of 10 the grid openings of the grid member. Such a construction enhances strength of the grid member and plugging strength of the structural filler which plugs mesh openings of the mesh.

In another modified form, the first reinforcing elements and the second reinforcing elements may have a substantially rectangular cross-section.

In practice, the grid member may be substantially 15 two-dimensional and be embedded in the structural component body so that it is parallel with a surface of the latter.

Further, the grid member may be used in the number of at least two, and adjacent grid members may be disposed to overlap each other at peripheral portions thereof.

Preferably, the first textiles may be each formed into 20 at least one structure of a tow, roving, strand, yarn, thread, sennit, twisted cord and braid, and may be made of at least one fiber selected from the group consisting of a glass fiber, carbon fiber, aramid fiber, boron fiber, 25 ceramic fiber, and metallic fiber. The structural filler may be a substance selected from the group consisting of a concrete, cement, plaster, glass, clay, mixture of both a clay and pieces of a straw, carbon, asbestos, epoxy resin, unsaturated polyester resin, vinyl ester resin, polyurethane resin, diallylphthalate resin, phenol formaldehyde resin, polyacetal resin, saturated polyester resin, unsaturated polyester resin, ABS (acrylonitrile butadien styrene copolymer), polyimide, polyamide 30 resin, polystyrene resin, polycarbonate resin, polyvinyl chloride resin, polyethylene resin, polypropylene resin, acrylic resin, PEEK (polyetheretherketone), PPS (polyphenylene sulfide) and like material.

The first resin matrixes are preferably made of a substance selected from the group consisting of an epoxy resin, unsaturated polyester resin, vinyl ester resin, polyurethane resin, diallylphthalate resin, phenolic plastic, polyacetal, saturated polyester resin, polyamide resin, polystyrene resin, polycarbonate resin, polyvinyl chloride resin, polyethylene resin, polypropylene resin and acrylic resin.

Preferably, the first reinforcing elements and the second reinforcing elements each contain about 10 to about 90% by volume of the first textiles and about 90 to about 10% by volume of the first resin.

In another preferred form, the first reinforcing elements and the second reinforcing elements each contain about 30 to about 70% by volume of a glass fiber and about 70 to about 30% by volume of a vinyl ester resin.

In still another preferred form, the first reinforcing elements and the second reinforcing elements each contain about 20 to 60% by volume of a carbon fiber and about 80 to about 40% by volume of a vinyl ester resin.

Preferably, the textile reinforced structural component may further comprise: at least three longitudinal parallel reinforcing elements disposed in a three-dimensional manner; and second attaching means for attaching the longitudinal parallel reinforcing elements to the

first reinforcing elements and the second reinforcing elements, and wherein the first reinforcing elements and the second reinforcing elements cross corresponding longitudinal reinforcing elements at second crossing portions and are attached to the corresponding longitudinal reinforcements at second crossing portions with the second attaching means. Such a construction provides a three-dimentional reinforcement unit having an excellent strength, workability, and transportability as compared to the prior art reinforcement.

In a further preferred form, the longitudinal reinforcing elements may each comprise: at least one row of second parallel textiles; and a second resin matrix, made of a second resin, for integrally bonding the row of the second textiles. The textile rows of each of a corresponding first reinforcing element, a corresponding second reinforcing element and a corresponding longitudinal reinforcing element may be alternately stacked at each of the second crossing portions. The second attaching means may be one of the first resin and the second resin. With such a construction, the reinforcement unit may have the first reinforcement elements, the second reinforcement elements and the longitudinal reinforcement elements placed substantially at an equal level around the second crossing portions. Thus, substantially uniform structural filler covering depth may be achieved for the textile reinforced structural component. Further, the reinforcement unit provides sufficient strength to the textile reinforced structural component with fairly small thickness as compared to the prior art.

Further, the first reinforcing elements and the second reinforcing elements preferably extend between two adjacent longitudinal reinforcing elements so that the first reinforcing elements and the second reinforcing elements each generally define a spiral in the overall shape thereof.

The second textiles may be each formed into at least one structure of a tow, roving, strand, yarn, thread, sennit and braid, and wherein the second textiles are each made of at least one fiber selected from the group consisting of a glass fiber, carbon fiber, aramid fiber, boron fiber, ceramic fiber, and metallic fiber. The structural filler may be a substance selected from the group consisting of a concrete, cement, plaster, glass, clay, mixture of both a clay and pieces of a straw, carbon, asbestos, an epoxy resin, unsaturated polyester resin, vinyl ester resin, polyurethane resin, diallylphthalate resin, phenolic resin, polyacetal resin, saturated polyester resin, polyamide resin, polystyrene resin, polycarbonate resin, polyvinyl chloride resin, polyethylene resin, polypropylene resin, acrylic resin, and polyetheretherketone. Further, the second resin matrixes may each be made of a substance selected from the group consisting of an epoxy resin, unsaturated polyester resin, vinyl ester resin, polyurethane resin, diallylphthalate resin, phenolic plastic, polyacetal, saturated polyester resin, polyamide resin, polystyrene resin, polycarbonate resin, polyvinyl chloride resin, polyethylene resin, polypropylene resin and acrylic resin.

The longitudinal reinforcing elements may each contain about 10 to about 90% by volume of the second textiles and about 90 to about 10% by volume of the second resin. Preferably, the longitudinal reinforcing elements each contain about 30 to about 70% by volume of a glass fiber and about 70 to about 30% by volume of a vinyl ester resin. In another preferred form, the longitudinal reinforcing elements each contain about 20 to

60% by volume of a carbon fiber and about 80 to about 40% by volume of a vinyl ester resin.

#### BRIEF DESCRIPTION OF THE DRAWINGS

5 The invention will now be described by way of example with reference to the accompanying drawings in which:

10 FIG. 1 is a perspective view of a concrete reinforcing unit used in a concrete panel according to the present invention;

15 FIG. 2 is an enlarged cross-section of each of the first reinforcing elements and the second reinforcing elements in FIG. 1;

20 FIG. 3 is an enlarged cross-section of a crossing portion in FIG. 1;

25 FIG. 4 is a plan view of an apparatus for fabricating the concrete reinforcing unit in FIG. 1, with the first and the second reinforcing elements set in it;

30 FIG. 5 is a side view of the apparatus in FIG. 4 with a depressing plate placed in position;

35 FIG. 6 is an illustrative view demonstrating how to interweave resin-impregnated textile rows to produce the concrete reinforcing unit in FIG. 1;

40 FIG. 7 is an enlarged cross-sectional view of one of the resin-impregnated textile bundles before it is depressed with the depressing plate in FIG. 5;

45 FIG. 8 is an enlarged cross-sectional view of the depressed textile bundle in FIG. 7;

50 FIG. 9 is a perspective view of a concrete reinforcing unit having a lattice girder structure and used in a concrete column or beam according to the present invention;

55 FIG. 10 is an enlarged partial view of the concrete reinforcing unit in FIG. 9;

60 FIG. 11 is an enlarged cross-section of each of the spiral reinforcing elements and the longitudinal reinforcing elements;

65 FIG. 12 is an enlarged cross-section taken along the line XII—XII in FIG. 10;

70 FIG. 13 is an enlarged cross-section taken along the line XIII—XIII in FIG. 10;

75 FIG. 14 is a front view of an apparatus for fabricating the concrete reinforcing unit in FIG. 9;

80 FIG. 15 is an enlarged view taken along the line XV—XV in FIG. 14;

85 FIG. 16 is an enlarged partial view of the apparatus in FIG. 14 with the spiral elements and the longitudinal elements crossing each other;

90 FIG. 17 is an enlarged view, partly in axial section, of the hooking portion of the apparatus in FIG. 14;

95 FIG. 18 is an illustration with a two-dimensional expansion as to how to interweave the spiral elements and the longitudinal elements;

100 FIG. 19 is a plan view of a concrete panel used in Example 1, the upper grid shown by the solid lines for illustration purpose;

105 FIG. 20 is a side view of the concrete panel in FIG. 19;

110 FIG. 21 is a plan view of another concrete panel used in Comparative Test, the upper grid shown by the solid lines for illustration purposes;

115 FIG. 22 is a front view of a test piece of Example 1 placed in a test machine; and

120 FIG. 23 is a graph showing results of a static load tests.

125 FIG. 24 is a perspective view, partly broken away, of a hemispherical shell structure of which the dome portion is constructed according to the present invention;

FIG. 25 is an enlarged, fragmentary, perspective view, partly broken away, of the dome portion of the hemispherical shell in FIG. 24;

FIG. 26 is a further enlarged perspective view of part of the reinforcing unit in FIG. 25;

FIG. 27 is a perspective view, partly broken away, of a concrete column constructed according to the present invention, with only part of the meshes shown for illustration;

FIG. 28 is a perspective view, partly broken away, of a body of a fiber-reinforced plastic boat constructed according to the present invention, with the meshes omitted for illustration purpose;

FIG. 29 is a plan view, partly broken away, of a transparent floor block constructed according to the present invention; and

FIG. 30 is a view taken along the line XXX—XXX in FIG. 29.

#### DETAILED DESCRIPTION OF THE PREFERRED EMBODIMENTS

The textile reinforced structural component according to the present invention includes, for example, a textile reinforced roof, wall, girder and column of a concrete or wooden construction, a transparent block 25 of a building, and a body of a fiber-reinforced plastic boat.

FIGS. 1 to 3 illustrate a concrete reinforcing unit 30 in the shape of a grid used in the present invention. The reinforcing unit 30 is suitably used as a reinforcement which is embedded in concrete to form a wall or a floor of a building. The reinforcing unit 30 includes a plurality of first parallel reinforcing elements 32 and a plurality of second parallel reinforcing elements 34 crossing the first parallel reinforcing elements 32 to form a grid, 35 all the first and second reinforcing elements 32 and 34 being disposed in a plane. In this embodiment, the number of the first reinforcing elements 32 is five and the number of the second reinforcing elements 34 is four. As illustrated in FIG. 2, each of the first and second reinforcing elements 32 and 34 includes eight vertically stacked rows 40 of textiles 36 which are bonded together through a resin matrix 38. Each textile row 40 has four parallel textiles 36, rovings in this embodiment, contacting or nearly contacting adjacent textile or textiles 36 of the same row 40. Crossing portions 42 of both the first and second reinforcing elements 32 and 34 is illustrated in a sectional view in FIG. 3, in which eight textile rows 40 of the first reinforcing elements 32 and eight textile rows 40 of the second reinforcing elements 34 are alternately stacked, so that the crossing portion 42 has 16 rows of textiles in total in this embodiment. However, the number of textile rows 40 in each crossing portion 42 may be two or more. Each crossing portion 42 and non-crossing portions of the first and second reinforcing elements 32 and 34 are substantially equal in thickness T. Hence, the upper and lower faces of the reinforcing unit 30 are each at an equal level. The upper and lower faces of the reinforcing unit 30 may be roughened for enhancing adhesive strength to the resin of the resin matrix 38.

In the present invention, the structure of the textiles 36 include, for example, a tow, roving, strand, yarn, thread and braiding.

Textiles 36 are, according to the present invention, made of: for example, a glass fiber; carbon fiber; aramid fiber; boron fiber; ceramic fiber such as made of alumina, silica and titanium oxide; metallic fiber such as

stainless steel fiber; and combination thereof. Preferably, glass fiber and carbon fiber are used due to relatively light weight and high strength.

The resin matrix 38 which bonds textile rows 40 together is, according to the present invention, preferably made of a vinyl ester resin due to its excellent adhesiveness to textiles 36 and sufficient strength. However, the resin forming the resin matrix 38 depends on the kind of textiles used. Use may be made of other synthetic resins such as an epoxy resin, unsaturated polyester resin, polyurethane resin, diallylphthalate resin, phenolic plastic, polyacetal, saturated polyester resin, polyamide resin, polystyrene resin, polycarbonate resin, polyvinyl chloride resin, polyethylene resin, polypropylene resin and acrylic resin.

The reinforcing unit 30, according to the present invention, generally contains about 10 to about 90% by volume of the textile 36. However, the ratio is selected in view of the kind and strength of the textiles 36 and use of the reinforcing unit. When a glass fiber is used for the textiles 36 and a vinyl ester resin is used for the resin matrix 38, the reinforcing unit 30 for building constructions includes preferably about 30 to about 70% by volume of the glass fiber. Below about 30%, strength of the resultant reinforcing unit reduces, and above about 70%, the resulting reinforcing unit is costly in the glass fiber. When a pitch carbon fiber and a vinyl ester resin are used, the reinforcing unit includes preferably about 20 to about 60% by volume of the pitch carbon fiber. Below about 20% by volume of the pitch carbon fiber, the resulting reinforcing unit is rather inferior in strength, and above about 60%, cost performance of the carbon fiber is considerably reduced—although the reinforcing unit has relatively high strength.

The reinforcing unit 30, according to the present invention, may be produced by means of an apparatus as illustrated in FIGS. 4 and 5, although in this apparatus a grid reinforcing unit having five first reinforcing elements 32 and nine second reinforcing elements 34 is to be fabricated. In FIGS. 4 and 5, the reference numeral 50 designates a rectangular base plate having chamfered upper edges 52. Tapered pins 54 are mounted in the number of 28 at their smaller diameter ends to lateral faces 56 of the base plate 50 so that they are located to correspond to pitches of the first and second reinforcing elements 32 and 34.

In producing the reinforcing unit 30, a row 60 of continuous textiles 62, which are impregnated with a resin for forming the resin matrix 38, are hooked around each pin 54 to extend it tightly between facing pins 54, for example, in a longitudinal direction L and then in a transverse direction T in the order I-XXVIII as shown in FIG. 4. When a grid member having more than two textile rows 40 is made as in this embodiment, the row 55 of the continuous textiles 62 is returned from the pin XXVIII to the pin I and then the operation described above is repeated. Adjacent textile rows 60 and 60 at crossing portions 42 cross each other. That is, textile rows example 1 of the first and second reinforcing elements 32 and 34 are alternately stacked at the crossing portions 42. FIG. 6 illustrates one crossing portion 42 of four rows 60 of textiles 62 impregnated with a resin, each textile row 60 including four textiles 62, rovings in this embodiment. The four textile rows 60 are stacked in the alphabetical order A-D as illustrated. Thus, in the reinforcing unit 30 in FIGS. 1 to 3, the above-stated operation which consists of four steps A to D is repeated four times, since each crossing portion 42 thereof

includes 16 rows vertically stacked. In this process sufficient tension must be applied to the textiles 62 to keep them tight. This process may be manually carried out, or it may be achieved automatically by means of a numerically controlled machine which is actuated on a predetermined program describing a two-dimensional pattern of the grid member 30. Then, the reinforcing unit thus formed (FIG. 7) is depressed by means of a depressing plate 64 as shown in FIG. 8 for providing a uniform thickness to it. When the resin is set, each of the first and the second reinforcing elements 32 and 34 is cut at their opposite ends near the pins 54 and then removed from the base plate 50. Thus, the grid member 30 is completed. It is to be noted that the base plate 50 and the depressing plate 64 should have poor adhesive properties to the resin. In this embodiment, the working faces of the base plate 50 and the depressing plate 64 are coated with Teflon resin, and a wax is applied to the pins 54 for this purpose.

Rough surfaces may be formed in the upper or lower faces of the reinforcing unit 30 by providing irregularity to the lower face of the depressing unit 64 or the upper face of the base plate 50. The rough faces of the reinforcing unit 30 enhances its adhesive property to the concrete in which it is embedded.

Although two adjacent first reinforcing elements 32 and 32 and two adjacent second reinforcing elements 34 and 34 define a square pattern, they may form a diaper pattern. The grid member 30 may have bias reinforcing elements crossing both the first and second reinforcing elements 32 and 34. In this case, a reinforcing unit 30 having a hexagonal pattern may be formed. In this embodiment, the reinforcing unit 30 has a constant pitch, but a portion of the reinforcing unit 30 may have a pitch larger than the other portion, in which case a rectangular pattern may be defined.

For producing a grid reinforcing unit, a plurality of separate first and second reinforcing elements previously set may be attached. In this case, the separate first and second reinforcing elements are bound with strings or fastened with bolts and nuts at the crossing portions. Alternatively, they may be bonded or attached by melting.

FIGS. 9 and 10 illustrate another concrete reinforcement unit 70 having a lattice girder structure according to the present invention. The reinforcement unit 70 is used as a reinforcement for a column or a beam of a concrete building. The reinforcement unit 70 includes four parallel longitudinal reinforcing elements 72, four first spiral reinforcing elements 74 as lattice bars, and four second spiral reinforcing elements 76 as the other lattice bars. The longitudinal reinforcing elements 72 are disposed in a three-dimensional manner with an equal spacing. The first spiral reinforcing elements 74 and the second spiral reinforcing elements 76 spirally extend around the four longitudinal reinforcing elements 72 in opposite directions, thus forming crossing portions A on longitudinal reinforcing elements 72 and crossing portions B between adjacent two longitudinal reinforcing elements 72 and 72. As illustrated in FIG. 11, each of the longitudinal reinforcing elements 72 and the spiral reinforcing elements 74, 76 has a structure similar to the structure, as shown in FIG. 2, of the reinforcing elements 32 and 34 of the reinforcing unit 30. However, each of the longitudinal reinforcing elements 72 and the spiral reinforcing elements 74, 76 includes four textile rows 80, and each row 80 consists of five textiles 36. The textiles of these elements 72, 74 and 76

may be the same in their material and structure as the textiles of the reinforcing unit 30, and they are contained in a resin matrix 82 which may also be made of the same material as the resin matrix 38 of the preceding embodiment. In this embodiment, the textiles 36 of each of the longitudinal reinforcing elements 72 and the first and second spiral reinforcing elements 74 and 76 are integrally bonded by the resin matrix 82 of the same resin. The longitudinal reinforcing elements and the first and second spiral reinforcing elements are substantially equal in the ratio of the textiles over the resin to those of the first embodiments.

In each of the crossing portions A, textile rows 80 of a corresponding longitudinal reinforcing element 72 and corresponding first and second spiral reinforcing elements 74 and 76 are, as illustrated in FIG. 12, alternatively stacked to form at least three stacked rows, twelve rows in this embodiment. Each of the crossing portions B have textile rows 80 of the first and the second spiral reinforcing elements 74 and 76 alternately stacked in the same manner as the crossing portions 42 of the reinforcing elements 32 and 34 of the reinforcing unit 30 shown in FIG. 3. However, in this embodiment the total number of the textile rows 80 stacked in eight, 20 with each row 80 including five textiles 36. The thickness T of each of the longitudinal reinforcing elements 72 and the first and second spiral reinforcing elements 74 and 76 is substantially equal.

The concrete reinforcement unit 70 is fabricated by means of an apparatus illustrated in FIGS. 14 and 15, in which the reference numeral 90 designates a rotation shaft. Opposite ends of the rotation shaft 90 are rotatably supported on a pair of bearing stands 92 through ball bearings (not shown). The rotation shaft 90 has six sets of equidistant supporting arms 94. Each set includes four supporting arms 94 projecting radially outwardly from the rotation shaft 90 at equal angular intervals i.e., 90°. The supporting arms 94 are disposed so that they are axially aligned for forming four axial rows of supporting arms 94 as shown in FIG. 15. As best shown in FIG. 17, each supporting arm 94 includes a supporting pipe 96 fixed at its proximal end to the rotation shaft 90, a nut member 98 rotatably supported on the distal end of the supporting pipe 96, and a two-pronged hook member 100 threaded to the nut member 98. Each supporting pipe 96 has an inner circular flange 102 formed by bending its distal end radially inward, and the circular flange 102 fits in a circular groove 104 formed in the associated nut member 98 for supporting the nut member 98. The two-pronged hook members 100 each have a stem portion 106 and a two-pronged hook portion 108 formed integrally with one end of the stem portion 106. The stem portion 106 of each hook member 100 is threaded with the nut member 98, and thus rotation of the nut member 98 axially moves the hook member 100 by preventing rotation of the latter.

In production, a row 80 of continuous resin-impregnated textile 36 is prepared by passing it through a bath of a resin, vinyl ester resin in this embodiment. Then, it is hooked under tension manually in hook portions 108 of hook members 100 of the supporting arms 94 in sequence to define the reinforcement unit 70. FIG. 18 illustrates a sequence of hooking the textile row 80 in development elevation, in which the two phantom lines indicate the same portion to form a longitudinal reinforcing element 72, and the arrows show the directions of passing of the textile row 80. The hooking of the textile row 80 starts from a supporting arm 94 which is,

for example, one supporting arm 94, designated by O, of the leftmost support arm set in FIG. 14. The textile row 80 passes through the hook portion 108 of each hook member 100 in the numeric sequence given in FIG. 18 and then returns to its start point O. FIG. 16 illustrates a crossing portion A at this time. In this embodiment, this procedure is repeated four times. The textile row 80 thus extended must be kept tight until the impregnated resin is set. After setting of the resin, portions of the continuous textile, shown by the broken lines in FIG. 18, are cut. Next, the nut member 98 of each supporting arm 94 is turned to retract the stem portion 106 of the hook member 100 toward the supporting pipe 96 for separating the crossing portions A thus set from the associated hook members 100. By this operation the concrete reinforcement unit 70 is removed from the apparatus shown in FIG. 14 and completed.

The process above stated may be achieved automatically by means of a conventional numerically controlled machine which is actuated on a predetermined program describing the three-dimensional pattern of the concrete reinforcement unit 70.

When the thickness of the longitudinal reinforcing elements 72 must be larger, an additional resin-impregnated textile row or rows are added to the portions to form them. The three-dimensional concrete reinforcement unit according to the present invention is not limited to a square tubular, but may be in the shape of a rectilinear tube, quadrangular pyramid, hollow cylinder, cone or other like configurations. The pitch of the crossing portions A of a longitudinal reinforcing element or elements 72 may be partially changed. Further, the reinforcing unit 70 may have an additional reinforcing element or elements such as a hoop.

The reinforcing units 30 and 70 are embedded in structural component bodies made of a structural filler.

Although the structural filler according to the present invention depends on its field of use, it includes, for example, a water-hardenable material, such as a concrete, mortar and plaster, glass, carbon, asbestos, and various kinds of synthetic resins such as an epoxy resin, unsaturated polyester resin, vinyl ester resin, polyurethane resin, diallylphthalate resin, phenol formaldehyde resin, polyacetal resin, saturated polyester resin, unsaturated polyester resin, ABS (acrylonitrile butadien styrene copolymer), polyimide, polyamide resin, polystyrene resin, polycarbonate resin, polyvinyl chloride resin, polyethylene resin, polypropylene resin, acrylic resin, PEEK (polyetheretherketone) and PPS (polyphenylene sulfide). The concrete may include a conventional cement such as portland cement and other cements and the ratios of cement:water:sand:aggregate; and other components may be varied within the usual limits used for concrete structures. Further, a clay and a mixture of a clay and pieces of a straw may be used as the structural filler for a textile reinforced clay wall or roof constructed according to the present invention.

FIG. 24 illustrates a hemispherical shell with a dome 200 constructed according to the present invention. The dome 200 uses modified reinforcing units 202 similar to the reinforcing unit 30 in FIG. 1. Each reinforcing unit 202 is distinct from the reinforcing unit 30 in that it includes additional mesh 204 formed in each grid opening 206 which is defined with adjacent first and second parallel reinforcing elements 32 and 34. Each mesh 204 includes first parallel resin impregnated mesh textiles 210 and second parallel resin impregnated mesh textiles 212, the textiles 210 and 212 being stacked at crossing

portions. The pitch of the additional meshes 204 is selected for adhesion of a concrete mortar to be sprayed to it. When the reinforcing unit 202 is produced, the first resin impregnated textiles 210 may be continuous to the textiles 36 of the first parallel reinforcing elements 32 and pass through the second parallel reinforcing elements 34, while the second resin impregnated textiles 212 may be continuous to the textiles 36 of the second parallel reinforcing elements 34 and pass through the first parallel reinforcing elements 32. Each of the first and second textiles 210 and 212 may include a row of textile elements, and such textiles may be stacked as illustrated in FIGS. 1 and 2.

Reinforcing units 202 thus prepared are attached to beams 214 of the dome 200 to extend between adjacent beams 214, thus forming a dome frame structure 203 as illustrated in FIG. 24. A concrete mortar 216 is, as shown in FIG. 25, sprayed over the meshes 204 of these reinforcing units 202 to form a ceiling construction 217.

For relatively small-sized shell buildings (for example, shell structure houses) which are built in a little rain area, a clay or a like material may be used for the structural filler in place of the concrete mortar 216.

FIG. 27 illustrates a concrete column 220 constructed according to the present invention, in which the reinforcing unit 202 is formed into a rectangular tube 221 and embedded in a concrete 222. A motor may be applied over the outer faces of the reinforcing unit 202.

Another embodiment of the present invention is shown in FIG. 28, in which the reinforcing unit 202 is used for a fiber-reinforced plastic boat 230. In this embodiment, the body of the boat 230 is constructed with the reinforcing unit 202. A liquid of a conventional synthetic resin 232 which is used for the conventional fiber-reinforced plastic boat is applied over the reinforcing unit 202 to form the component body after it is set. Although in FIG. 28 additional meshes 204 are not shown, their pitch or mesh may be selected so that the synthetic resin liquid does not drip through the mesh openings.

FIGS. 29 and 30 illustrate a transparent floor block 240 constructed according to the present invention. The block 240 constitutes part of the partition between the upper and lower floor. The block 240 has a square reinforcing unit 30 embedded in a transparent synthetic resin 242 such as an acrylic resin and methacrylic resin. This block 240 is formed by supplying the synthetic resin 242 in molten state into a mold in which the reinforcing unit 30 is placed in position. The block 240 is fitted into an opening formed through a floor 244, so that light is allowed to pass through it.

#### EXAMPLE 1

A 200 mm × 100 mm × 1000 mm concrete panel which had a pair of glass fiber meshes 110 and 110 placed horizontally within it was prepared as illustrated in FIGS. 19 and 20, in which one mesh is shown by the solid line for illustration purposes. The pitch of each of the meshes was 100 mm and length, and the width thereof were 600 mm and 200 mm respectively. The projected portions 116 of crosswise elements 112 and longitudinal elements 114 of the meshes were 50 mm long. Although the outer ends 118 and 118 of longitudinal elements 114 and 114 of each mesh were continuous via connecting element 120, it is believed that this resulted in no substantial influence on the experimental results. The two meshes were overlapped 150 mm at their inner end portions in contact with each other. The

distance from the lower face of the lower mesh 110 to the bottom of the concrete panel was 20 mm.

Each of the glass fiber meshes 110 and 110 has substantially the same cross-sectional structure even in crossing portions thereof as the grid member 30 shown in FIGS. 1 to 3. That is, each of both crosswise elements 112 and the longitudinal elements 114 of the meshes had vertically stacked eight rows of glass fiber rovings bonded with a vinyl ester resin, each row consisting of four rovings. The vinyl ester resin was sold by Nippon (Japan) Upica, Japan under the trade designation "8250". Both the lengthwise and crosswise elements have substantially equal cross-sectional areas of about 10 mm × 10 mm. Each roving consisted of about 2,100 glass fiber filaments, each of which had a diameter about 23 micrometers, a density of 2.55 g/cm<sup>3</sup>, and denier of 19,980. Properties of the lengthwise and crosswise elements of the glass fiber meshes are given in TABLE 1. The average tensile strength of these elements was determined by stretching 200 mm long test pieces with their opposite end portions 50 mm long, cramped through a glass fiber roving cloth with chucks. The average strength of the crossing portions of the grid was determined by the use of cross-shaped test pieces 129 cut from the grid, as shown in FIG. 22, having a width 80 mm and a length 90 mm. Each test piece 129 was fitted at its one longitudinal leg 30 mm long into a hole 130 formed in a base 132 of a test machine. Static loads were vertically applied to the upper end of the other longitudinal leg 50 mm long. The strength of the crossing portions is defined as a shear fracture load of the crosswise legs/the effective cross-sectional area of the legs. The results are also given in Table 1. The properties of the concrete used are set forth in Table 2.

The concrete panel thus prepared was cured and then placed on a pair of parallel supporting rods 136 and 136 for determining its load-strain behavior so that each rod 136 was located 280 mm away from the center of the panel. Then, a depressing plate 138 having a pair of parallel depressing rods 140 and 140 welded at its bottom face 280 mm away from each other was placed on the upper face of the concrete panel so that each depressing rod 140 was located 140 mm away from the center of the panel. Thereafter, static loads were applied to the depressing plate 138, and the results are plotted with the solid line in FIG. 23. It was noted that longitudinal elements 114 were fractured at the point P1.

## EXAMPLE 2

Another concrete panel having a pair of carbon fiber grids placed within it was prepared and cured. The shape and size of the concrete panel and the grids were substantially the same as those in Example 1, and the carbon fiber grids were disposed in the concrete panel also in the same manner as in FIGS. 19 and 20.

The cross-sectional structure of each of the lengthwise and crosswise elements was substantially the same as that of each of the lengthwise and crosswise elements in Example 1 even in crossing portions except that each row of carbon fiber rovings included five rovings, each containing 10,000 carbon monofilaments having about 8 micrometers diameter. The carbon fiber roving elements were bonded with the same vinyl ester resin as in Example 1. The properties of the elements of the grid were determined by the same procedures in Example 1, and the results are given in Table 1. The carbon grid reinforced concrete panel underwent the same load-

strain test as in Example 1, and the results are also plotted with the broken line in FIG. 23. It was noted that longitudinal elements were fractured at the point P2.

## COMPARATIVE TEST

A steel grid reinforced concrete panel was prepared as illustrated in FIG. 21. The steel grid reinforced concrete panel had the same size and structure as in Example 1 except that the longitudinal outer end portions of lengthwise elements of each grid were straight and not jointed together, and that the lengthwise and crosswise elements had a diameter 9.53 mm.

The steel grid reinforced concrete panel was subjected to the same load-strain test as in Example 1, and the results are also plotted with the phantom line in FIG. 23. It was noted that welded points of the crossing portions of the lengthwise and crosswise elements were fractured at the point P3.

TABLE 1

|                                                             | (average values given) |      | Comparative<br>Test 1 |
|-------------------------------------------------------------|------------------------|------|-----------------------|
|                                                             | Example<br>1           | 2    |                       |
| Effective Cross-<br>sectional area (mm <sup>2</sup> )       | 70.8                   | 88.4 | 71.3                  |
| Content of fiber<br>in grid (volume %)                      | 39.4                   | 22.6 | —                     |
| Tensile strength<br>(kg/mm <sup>2</sup> )                   | 72.1                   | 38.1 | 57.0                  |
| Young's modulus<br>(kg/mm <sup>2</sup> )                    | 2800                   | 7400 | 19000                 |
| Strength of cross-<br>ing portions<br>(kg/mm <sup>2</sup> ) | 26.1                   | 16.3 | 15.8                  |

TABLE 2

| Compressive<br>Strength<br>(Kg/cm <sup>2</sup> ) | Young's<br>Modulus<br>(ton/cm <sup>2</sup> ) | Poisson<br>Ratio | Fracture<br>Strength<br>(Kg/cm <sup>2</sup> ) |
|--------------------------------------------------|----------------------------------------------|------------------|-----------------------------------------------|
| 272-310                                          | 255-285                                      | 0.16-0.18        | 27-34                                         |

What is claimed is:

1. A textile reinforced structural component comprising:
    - (a) a structural component body made of a structural filler;
    - (b) first parallel reinforcement elements;
    - (c) second parallel reinforcement elements crossing said first parallel reinforcement elements at first crossing portions, each of both said first reinforcement elements and said second reinforcement elements including at least one row of first textiles and a first resin matrix, made of a first resin, for bonding said first textiles thereof; and
    - (d) attaching means for attaching said first reinforcement elements and said second reinforcement elements at corresponding first crossing portions to form a grid member, said attaching means comprising said first resin,
- wherein:
- (e) said first and said second reinforcement elements are impregnated with said first resin before attachment thereof;
  - (f) said grid member is embedded in said structural component body;
  - (g) at least one of both said first reinforcement elements and said second reinforcement elements each comprise a plurality of textile rows;

- (h) the textile rows of both a corresponding first reinforcement element and a corresponding second reinforcement element are alternately stacked at said first crossing portions,
- (i) said first reinforcement elements and said second reinforcement elements are bonded with said first resin at said first crossing portions;
- (j) said grid member includes a plurality of grid openings; and
- (k) said textile reinforced structural component further comprises first resin impregnated mesh textiles and second resin impregnated mesh textiles, each of said first and second resin impregnated mesh textiles passing through at least one of both said first reinforcement elements and said second reinforcement elements to form a mesh in each of said grid openings.

2. A textile reinforced structural component as recited in claim 1, wherein said first reinforcement elements and said second reinforcement elements have a substantially rectangular cross-section.

3. A textile reinforced structural component as recited in claim 2, wherein:

- (a) said grid member is substantially two-dimensional and
- (b) said grid member is embedded in said structural component body so that said grid member is parallel with a surface of said structural component body.

4. A textile reinforced structural component as recited in claim 3, wherein:

- (a) said grid member has a peripheral portion;
- (b) said grid member is used in the number of at least two; and
- (c) adjacent grid members are disposed to overlap each other at the peripheral portions thereof.

5. A textile reinforced structural component as recited in claim 1, 2, 3 or 4, wherein:

- (a) said first textiles are each formed in at least one structure of a tow, roving, strand, yarn, thread, sennit, twisted cord, and braid;
- (b) said first textiles are made of at least one fiber selected from the group consisting of a glass fiber, carbon fiber, aramid fiber, boron fiber, ceramic fiber, and metallic fiber; and
- (c) said structural filler is a substance selected from the group consisting of a concrete, cement, plaster, glass, clay, mixture of both a clay and pieces of a straw, carbon, asbestos, an epoxy resin, unsaturated polyester resin, vinyl ester resin, polyurethane resin, diallylphthalate resin, phenolic resin, polyacetal resin, saturated polyester resin, unsaturated polyester resin, ABS (acrylonitrile butadiene styrene copolymer), polyimide, polyamide resin, polystyrene resin, polycarbonate resin, polyvinyl chloride resin, polyethylene resin, polypropylene resin, acrylic resin, PEEK and PPS.

6. A textile reinforced structural component as recited in claim 5, wherein said first resin matrixes are each made of at least one substance selected from the group consisting of an epoxy resin, unsaturated polyester resin, vinyl ester resin, polyurethane resin, diallylphthalate resin, phenolic resin, polyacetal resin, saturated polyester resin, polyamide resin, polystyrene resin, polycarbonate resin, polyvinyl chloride resin, polyethylene resin, polypropylene resin and acrylic resin.

7. A textile reinforced structural component as recited in claim 6, wherein said first reinforcement ele-

ments and said second reinforcement elements each contain about 10 to about 90% by volume of said first textiles and about 90 to about 10% by volume of said first resin.

8. A textile reinforced structural component as recited in claim 7, wherein said first reinforcement elements and said second reinforcement elements each contain about 30 to about 70% by volume of a glass fiber and about 70 to about 30% by volume of a vinyl ester resin.

9. A textile reinforced structural component as recited in claim 8, wherein said first reinforcement elements and said second reinforcement elements each contain about 20 to 60% by volume of a carbon fiber and about 80 to about 40% by volume of a vinyl ester resin.

10. A textile reinforced structural component as recited in claim 1, 2 or 3, and further comprising:

- (a) at least three longitudinal parallel reinforcement elements disposed in a three-dimensional manner and
- (b) second attaching means for attaching said longitudinal parallel reinforcement elements to said first reinforcement elements and said second reinforcement elements,
- (c) wherein said first reinforcement elements and said second reinforcement elements cross corresponding longitudinal reinforcement elements at second crossing portions and are attached to said corresponding longitudinal reinforcement elements at said second crossing portions with said second attaching means.

11. A textile reinforced structural component as recited in claim 10, wherein said longitudinal reinforcement elements each comprises:

- (a) at least one row of second parallel textiles and
- (b) a second resin matrix, made of a second resin, for bonding integrally said at least one row of said second textiles, p1 wherein:
- (c) the textile rows of each of a corresponding first reinforcement element, a corresponding second reinforcement element, and a corresponding longitudinal reinforcement element are alternately stacked at each of said second crossing portions and
- (d) said second attaching means is one of both said first resin and said second resin.

12. A textile reinforced structural component as recited in claim 11, wherein said first reinforcement elements and said second reinforcement elements extend between adjacent two longitudinal reinforcement elements so that said first reinforcement elements and said second reinforcement elements each define generally a spiral in an overall shape thereof.

13. A textile reinforced structural component as recited in claim 11, wherein:

- (a) said first textiles and said second textiles are each formed in at least one structure of a tow, roving, strand, yarn, thread, sennit, twisted cord, and braid;
- (b) said first textiles and said second textiles are each made of at least one fiber selected from the group consisting of a glass fiber, carbon fiber, aramid fiber, boron fiber, ceramic fiber, and metallic fiber; and
- (c) said structural filler is a substance selected from the group consisting of a concrete, cement, plaster, glass, clay, mixture of both a clay and pieces of a

straw, carbon, asbestos, an epoxy resin, unsaturated polyester resin, vinyl ester resin, polyurethane resin, diallylphthalate resin, phenolic resin, polyacetal resin, saturated polyester resin, polyamide resin, polystyrene resin, polycarbonate resin, polyvinyl chloride resin, polyethylene resin, polypropylene resin, acrylic resin, and polyetheretherketone.

14. A textile reinforced structural component as recited in claim 13, wherein said first resin matrixes and said second resin matrixes are each made of a substance selected from the group consisting of an epoxy resin, unsaturated polyester resin, vinyl ester resin, polyurethane resin, diallylphthalate resin, phenolic resin, polyacetal resin, saturated polyester resin, polyamide resin, polystyrene resin, polycarbonate resin, polyvinyl chloride resin, polyethylene resin, polypropylene resin and acrylic resin.

15. A textile reinforced structural component as recited in claim 14, wherein:

(a) said first reinforcement elements and said second reinforcement elements each contain about 10 to about 90% by volume of said first textiles and about 90 to about 10% by volume of said first resin and

(b) said longitudinal reinforcement elements each contain about 10 to about 90% by volume of said second textiles and about 90 to about 10% by volume of said second resin.

16. A textile reinforced structural component as recited in claim 15, wherein said first reinforcement elements, said second reinforcement elements, and said longitudinal reinforcement elements each contain about 30 to about 70% by volume of a glass fiber and about 70 to about 30% by volume of a vinyl ester resin.

17. A textile reinforced structural component as recited in claim 16, wherein said first reinforcement elements, said second reinforcement elements, and said longitudinal reinforcement elements each contain about 20 to 60% by volume of a carbon fiber and about 80 to about 40% by volume of a vinyl ester resin.

\* \* \* \* \*

25

30

35

40

45

50

55

60

65